

May 10, 1927.

1,628,017

M. M. WILCOX

TAPPET

Filed July 21, 1924



Fig. 1



Fig. 2



Fig. 3



Fig. 4

Inventor

Orrell M. Wilcox

By G. B. Wilcox

Attorney

Patented May 10, 1927.

## UNITED STATES PATENT OFFICE.

MERRILL M. WILCOX, OF SAGINAW, MICHIGAN; A. ELWOOD SNOW, ADMINISTRATOR OF SAID MERRILL M. WILCOX, DECEASED, ASSIGNOR, BY MESNE ASSIGNMENTS, TO WILCOX PRODUCTS CORPORATION, OF SAGINAW, MICHIGAN, A CORPORATION OF MICHIGAN.

## TAPPET.

Application filed July 21, 1924. Serial No. 727,338.

This invention relates to tappets and pertains more particularly to certain improvements in the construction and mode of operation of tappets made of cast iron, with 5 disk-like heads or platforms having hardened faces to receive the impacts of valve-actuating cams.

My present improvement has as an object to provide in the platform a means whereby 10 the depth of hardening of the chilled working face is made practically uniform throughout the entire area of the platform.

Further objects are to increase the strength 15 of the platform to withstand long continued percussions of the cam, and do it without materially increasing the weight of the tappet; also, by the same means to provide a platform construction that assists in more effective lubrication of the tappet stem as 20 it shoots to and from in the bore of the tappet bracket.

With the foregoing and certain other objects in view which will appear later in the specifications my invention comprises 25 the devices described and claimed and the equivalents thereof.

In the drawings Fig. 1 is a central vertical section of a chilled iron tappet head made in accordance with my invention.

30 Fig. 2 is a top plan view.

Fig. 3 is a central vertical section of a tappet as commonly produced heretofore showing faulty distribution of chill.

Fig. 4 is a fragmentary part sectional 35 view of one end of the tappet bracket showing the tappet in its raised position.

As is clearly shown in the drawings the tappet head is preferably made of a single piece of cast metal such as cast iron and 40 comprises two main parts, namely, the disk-like platform 1 and the integral shank or stem 2.

The platform has its working face 3 made flat or substantially so and hardened by 45 chilling in the mold. Its face is made smooth, preferably by grinding.

Upon the back of and cast integral with the platform is a reinforcing member, as, for example, the raised rim 4. The functions which this reinforcement performs are 50 of real importance, not only during the manufacture of the tappet, but also in its operation.

The working face 3 is made extremely

hard by chilling, as previously noted and it 55 is one of the functions of rim 4 to improve the effectiveness of chilling the molten metal in the mold, by making the depth of chill C practically uniform and of predetermined thickness over the entire area of platform 60 1, as indicated in Fig. 1.

Heretofore tappets made of cast iron have usually been formed as shown in Fig. 3, where the depth of chill at the rim of the platform, indicated by C', may be considerably greater than at the middle c'. The reason for such lack of uniformity in the depth of chill is that the mass of molten metal which forms the lower part of the central stem or shank, where it joins the 70 platform, is much greater than the mass at the edge portions of the platform. Consequently the edges of the platform, being thinner and therefore losing their heat more quickly, are chilled to a greater degree. 75 Frequently the smoothing of the face by grinding results in removing so much of the thinner chilled part of the metal at the center of the platform as to expose a relatively soft area in that part, whereas it 80 should be extremely hard. Various expedients have been devised to increase the depth of chill in the central area and make the entire surface uniform in that regard, 85 none of which attempts prior to my present invention have been entirely successful, so far as I am aware. I have found by long experimenting that a simple and inexpensive change in the configuration of the platform itself does entirely overcome the difficulty 90 and makes a stronger platform to resist impacts of the cam in the direction of the arrow, Fig. 3. My new construction also assists in improving the lubrication of the shank 2 in its bearing 5, as indicated in 95 Fig. 4.

I reduce the central mass of metal by eliminating the crowned back of the customary platform, shown in Fig. 3, and extend the shank 2 down to the flat top of the platform 1, as shown in Fig. 1. The reinforcing rim 4 or its equivalent supplies a sufficient body of molten metal at the edge of the platform to prevent its too rapid chilling. 100 The reduction of the mass of molten metal at the middle as above described, together with the increase of the mass of molten metal around the periphery of rim 4 has 105

the effect of establishing the depth of chill at the middle area of the platform and beneath the rim so that throughout the entire area of the working face a practically uniform depth is secured.

The rim 4 also acts as an oil collector which effectively splashes the oil over the rubbing surfaces of the tappet stem, thereby greatly increasing the effectiveness of lubrication of the stem in its bracket bearing 5.

Rim 4 also strengthens the tappet platform to resist impacts of the cam, since the rim serves as a reinforcing band or rib for the back of the platform. It has been found in practice that as compared with previous constructions such as in Fig. 3, the strength

to resist impacts against the face of the platform is fully fifty per cent greater in my improved construction, largely due to the more uniform depth of chill made possible 20 by the means herein set forth.

Having thus described my invention what I claim and desire to secure by Letters Patent is:

In a tappet having a shank and a platform cast integral and having the working face of said platform hardened by chilling, a raised reinforcing member cast integral 25 with the platform.

In testimony whereof, I affix my signature.

MERRILL M. WILCOX.